

## UNITED STATES PATENT OFFICE.

BERT BUHR, OF SUMNER, IOWA.

## POLISH.

No Drawing.

Application filed September 8, 1924. Serial No. 736,787.

*To all whom it may concern:*

Be it known that I, BERT BUHR, a citizen of the United States, residing at Sumner, in the county of Bremer and State of Iowa, 5 have invented certain new and useful Improvements in Polishes, of which the following is a specification.

The present invention appertains to a polish which is particularly efficient on automobile bodies, woodwork, pianos, furniture upholstery, hardwood floors, and the like. 10 The polish renews the luster of old paint and preserves the same. It can be manufactured and placed on the market at a comparatively 15 low cost and may be applied with the least amount of effort.

The composition consists of strained boiled linseed oil, pure sixty six test gasoline and boiled skunk oil. This skunk oil is 20 a very fine grade of oil which is gotten from the fat of a skunk. It is preferable to mix the ingredients in about the following proportions: In one quart of the polish there would be sixteen ounces of clean strained 25 boiled linseed oil, ten ounces of pure sixty six test gasoline and two ounces of boiled skunk oil.

The skunk oil takes away the sticky effect of the polish caused by the linseed oil. 30 Without this skunk oil, the polish is sticky and very hard to apply, but by adding this quantity of skunk oil it unites the other ingredients and eliminates all stickiness. The skunk oil also keeps the polish from forming 35 a hard surface while standing.

In using the polish to obtain the best results it is necessary to have the automobile body or the like perfectly clean and then the polish is applied as any ordinary polish after which it is rubbed until thoroughly 40 dry. It is best to use cheese cloth both for applying and rubbing the polish. If these directions are carried out it will be found that the polish will impart to an old paint job a new appearance with a brush luster 45 making the old paint look new and preserving the same. Of course, it is evident, that changes may be made in the preparation by varying proportions of the ingredients. It is also evident that the manner of using the 50 polish set forth above has been given by way of example and that applicant is not limited in any way as to the manner in which the polish may be used.

Having thus described my invention, what 55 I claim as new is:

1. A polish of the class described consisting of linseed oil, gasoline and skunk oil.
2. An automobile polish of the class described consisting of strained boiled linseed oil, pure sixty six test gasoline and boiled skunk oil. 60
3. A polish of the class described consisting of a plurality of ingredients mixed together in the following proportions, sixteen 65 ounces of clean strained boiled linseed oil, ten ounces of pure sixty six test gasoline and two ounces of boiled skunk oil.

In testimony whereof I affix my signature.  
BERT BUHR.